



US006534247B2

(12) **United States Patent**  
Milligan et al.

(10) **Patent No.:** US 6,534,247 B2  
(45) **Date of Patent:** Mar. 18, 2003

(54) **METHOD OF FABRICATING  
MICROMACHINED INK FEED CHANNELS  
FOR AN INKJET PRINthead**

(75) Inventors: **Donald J. Milligan**, Corvallis, OR (US); **Chien-Hua Chen**, Corvallis, OR (US)

(73) Assignee: **Hewlett-Packard Company**, Palo Alto, CA (US)

(\*) Notice: Subject to any disclaimer, the term of this patent is extended or adjusted under 35 U.S.C. 154(b) by 88 days.

(21) Appl. No.: **09/755,837**

(22) Filed: **Jan. 3, 2001**

(65) **Prior Publication Data**

US 2001/0002135 A1 May 31, 2001

**Related U.S. Application Data**

(60) Division of application No. 09/408,116, filed on Sep. 29, 1999, now Pat. No. 6,273,557, which is a continuation-in-part of application No. 09/033,987, filed on Mar. 2, 1998, now Pat. No. 6,162,589.

(51) **Int. Cl. 7** ..... **H01J 2/01**

(52) **U.S. Cl.** ..... **430/320; 216/2; 216/27**

(58) **Field of Search** ..... **430/320; 216/2, 216/27; 347/54, 56, 63, 65**

(56)

**References Cited**

**U.S. PATENT DOCUMENTS**

|                |        |                       |         |
|----------------|--------|-----------------------|---------|
| 4,894,664 A    | 1/1990 | Tsung Pan .....       | 346/1.1 |
| 5,308,442 A    | 5/1994 | Taub et al. .....     | 156/644 |
| 5,387,314 A    | 2/1995 | Baughman et al. ..... | 156/643 |
| 5,441,593 A    | 8/1995 | Baughman et al. ..... | 216/27  |
| 6,019,907 A *  | 2/2000 | Kawamura .....        | 216/27  |
| 6,209,993 B1 * | 4/2001 | Wang et al. .....     | 347/65  |

**FOREIGN PATENT DOCUMENTS**

|    |               |         |
|----|---------------|---------|
| EP | 0841167 A2    | 5/1998  |
| EP | 0 886 307 A * | 12/1998 |

\* cited by examiner

*Primary Examiner*—John A. McPherson

(57) **ABSTRACT**

An inkjet print cartridge comprising a printhead that is formed using a sequence of etch process steps is described. The first etch of the two etch step process is comprised of a wet chemical etch. A dry etch process follows. Both etch steps are consecutively initiated from the back of the wafer. The fabrication process described offers several advantages including precise dimensional control of the ink feed channel, greater packing density of ink ejectors disposed in the printhead and greater printing speed. Additionally, the time required to manufacture the printhead, in contrast to a conventional printhead, is reduced.

**19 Claims, 11 Drawing Sheets**





Fig. 1A



Fig. 1B



**Fig. 2**



Fig. 3A



Fig. 3B



Fig. 3C



Fig. 4A



Fig. 4B



Fig. 4C



Fig. 4D



Fig. 5A



Fig. 5B



Fig. 5C



Fig. 6A



Fig. 6B



Fig. 6C



Fig. 7A



Fig. 7B



Fig. 8A



Fig. 8B



**Fig. 9A**



**Fig. 9B**



**Fig. 10**



**Fig. 11A**



**Fig. 11B**



**Fig. 12A**



**Fig. 12B**

**METHOD OF FABRICATING  
MICROMACHINED INK FEED CHANNELS  
FOR AN INKJET PRINthead**

This invention is a divisional of application Ser. No. 09/408,116, filed on Sep. 29, 1999, now U.S. Pat. No. 6,273,557, which is a continuation in part of application Ser. No. 09/033,987, filed on behalf of Chien-Hua Chen, et al., on Mar. 2, 1998, now U.S. Pat. No. 6,162,589. This invention relates to an inkjet printhead and more specifically, to a method and apparatus for channeling ink from a reservoir to an ejecting nozzle.

**FIELD OF THE INVENTION**

**BACKGROUND OF THE INVENTION**

Thermal inkjet printers have experienced a great deal of commercial success since their inception in the early 1980's. The fundamental principles of how thermal inkjet printers work is analogous to what happens when a pot of coffee is made. Using the electric drip coffee maker analogy, water is poured into a container (reservoir) and is channeled towards a heating element that is located at the base of the container. Once the coffee has been placed in the filter, the coffee maker is turned on and power is supplied to the heating element that is surrounded by water. As the heating element reaches a certain temperature, some of the water surrounding it changes from a liquid to a gas, thus, creating bubbles within the water. As these "super heated" bubbles are formed, heated water surrounding these bubbles is pushed from the reservoir into a tube and finally into the carafe. Referring now to the thermal printhead, ink is located in a reservoir that has a heating element (heater resistor) at its base. When the heater resistor is turned on for a certain amount of time (pulsed by electronic circuitry) corresponding to a certain temperature, the ink surrounding the heater resistor changes from a liquid to gas phase, thus, creating a bubble that pushes surrounding ink through an orifice and finally onto a printing medium (carafe). The aforementioned example radically simplifies inkjet technology. For a more detailed treatment of the history and fundamental principles of thermal inkjet technology, refer to the *Hewlett-Packard Journal*, Vol. 36, No. 5, May 1985.

In the coffee maker analogy, the water was poured into a container (reservoir) and channeled to a heating element located at its base. This channeling, for an inkjet cartridge, may be accomplished in a variety of different ways with the objective being to simultaneously provide the ink ejecting heater resistors with a continuous supply of ink.

The ink channel has traditionally been a challenging feature to fabricate both in terms of manufacturing repeatability and manufacturing cost. When manufacturing a multiplicity of printheads, variation in critical dimensions can be cataclysmic. For example, if a channel's width is too narrow, it may restrict the flow of ink to the heater resistor(s) consequently causing variations in the volume of ink ejected onto the printing medium. Likewise, if the channel width is too large, ink may be more readily supplied to some heater resistors than others thus creating variations in the rate at which ink may be ejected from the printhead nozzles (hence, the distance through which ink travels before reaching the heater resistor impacts the speed/frequency at which the printhead operates).

In terms of cost, traditional techniques of fabricating ink feed channels involved "sand blasting" holes into a substrate as disclosed in U.S. Pat. No. 5,681,764. This technique,

although effective, required very specialized equipment that varied significantly from conventional IC processing thus requiring special facilities, personnel, and equipment. Consequently, there has been many efforts in the inkjet printing community to develop techniques for fabricating ink feed channels wherein the channel dimensions could be accurately controlled using standard IC manufacturing equipment and methodology. The following US patents describe such methods and techniques in an attempt to remedy the aforementioned problem.

U.S. Pat. No. 5,308,442 illustrates a method for isotropically etching ink feed channels employing wet chemical etching. This technique incorporates standard integrated circuit (IC) photolithography and wet etch processing methodology and provides an alternative to the traditional sand blasting approach. Additionally, it provides an improvement over the sand blasting technique wherein the path through which ink flows prior to reaching the heater resistor is shortened. This technique, however, is based purely on conventional anisotropic wet chemical etching (hereafter referred to as wet etching) from the backside of the wafer/wafer substrate subsequently limiting the dimensional control of the ink feed channel. The backside of the wafer refers to the side opposite of where nozzles will be formed.

U.S. Pat. No. 5,387,314 discloses a technique for channeling ink from a reservoir to a heater resistor by utilizing photolithography techniques with a combination of wet etching and plasma etching (a conventional gaseous etching technique hereafter referred to as dry etching). A semiconductor wafer, such as a silicon wafer, is used with a known crystallographic orientation to accommodate channels through which ink flows to the heater resistor. Such a wafer can be etched in two prominent process steps: Firstly, trenches are anisotropically etched part way into the semiconductor from the backside of the substrate. Secondly, an isotropic dry etch is used to etch from the front side (the side upon which nozzles are formed) of the substrate thus creating a channel through the substrate. The advantages of this technique as compared to that previously described in U.S. Pat. No. 5,308,442, is that the front side dry etch offers a greater degree of dimensional control. As this is well known in the semiconductor industry, isotropic wet etch processes are, in general, more variable than dry etch processes. Combining both dry and wet etch processing was a major step whereupon dimensional control of the ink feed channel was improved. However, the aforementioned process introduces an isotropic dry etch step from the front side of the wafer thus requiring the substrate above the ink feed channel to be void of active devices or signal lines.

Many of the aforementioned challenges associated with the fabrication of ink feed channels still persist. Consequently, there remains an opportunity to develop a manufacturing process and apparatus wherein: (1) ink feed channels dimensions can be precisely controlled, (2) the distance through which ink flows before reaching the heater resistor can be minimized, (3) and the time required to form the ink feed channel is reduced.

**SUMMARY OF THE INVENTION**

An inkjet print cartridge comprises a printhead which further comprises a substrate having at least one crystallographic orientation and opposed planar surfaces. A dielectric film is disposed on a first opposed substrate surface and a second opposed substrate surface. A first portion of the ink feed channel is formed commencing from the second opposed substrate surface and concluding between the

opposed substrate surfaces. A second portion of the ink feed channel is then etched commencing from the conclusion of the first etch thereby forming a channel completely through the substrate and terminating at the first disposed dielectric film. An opening positioned above the ink feed channel is formed in the dielectric film whereby ink flows through the channel from an ink reservoir. Additionally, the formation of the first portion of the ink feed channel may conclude at an etchstop disposed between the opposed planar surfaces.

#### BRIEF DESCRIPTION OF THE DRAWINGS

The present invention can be further understood by reference to the following description and attached drawings. Other features and advantages will be apparent from the following detailed description of a preferred embodiment taken in conjunction with the accompanying drawings which illustrate, by way of example, the principles of the invention.

FIG. 1A is a cross section of a conventional printhead showing a material stack which may comprise an ink ejecting apparatus of the printhead.

FIG. 1B is a perspective view of a printhead showing an ink feed channel and material stack.

FIG. 2 illustrates a print cartridge body to which the printhead is attached.

FIGS. 3A-3C shows views of a printhead that may use the present invention.

FIGS. 4A-4D show cross sectional views depicting a process sequence for forming the thinfilm hard mask and polymer layer.

FIGS. 5A-5C show cross sectional views depicting a process sequence for forming the first portion of the ink feed channel.

FIG. 6A shows a silicon substrate wherein the photoresist has been exposed so that the second portion of the ink feed channel can be defined.

FIGS. 6B-6C show a silicon substrate wherein the first and second portion of the ink feed channel have been etched thus providing a path for ink to travel from the inkjet cartridge to the heater resistor.

FIGS. 7A and 7B each show a preferred embodiment of the current invention wherein the thinfilm above the ink feed channel includes an ink filter.

FIG. 8A shows an embodiment of the present invention wherein the heater resistor is disposed in the thinfilm directly above the ink feed channel.

FIG. 8B shows an embodiment of the present invention wherein a multiplicity of heater resistors is disposed in the thinfilm directly above the ink feed channel.

FIGS. 9A-B show a printhead wherein the hard mask opening is substantially narrowed so that the crystallographic planes converge at a predetermined distance during the first etch.

FIG. 10 show a printhead wherein the first portion of the ink feed channel etch is conducted using an isotropic chemical etch.

FIGS. 11A-B show a printhead wherein the first surface of the silicon substrate is doped using a boron source in those regions where the ink feed channel is defined.

FIGS. 12A and 12B show a printhead fabricated on commercially available silicon on insulator substrate (commonly referred to as an SOI wafer).

#### DETAILED DESCRIPTION OF THE PREFERRED EMBODIMENTS

Many of the aforementioned challenges associated with the fabrication of ink feed channels have been resolved

through preferred embodiments of the present invention wherein both wet and dry etches are employed to define the ink feed channel. Unlike the process described in U.S. Pat No. 5,308,442, however, both processes are performed from the back side of a silicon wafer which is defined, hence forth, as the side of the wafer opposite to where ink is ejected onto a paper medium. This technique offers several advantages including greater alignment tolerances, shorter ink feed paths (allowing for a higher frequency printhead), selective positioning of the ink feed holes relative to the heater resistor, and significantly higher packing density of the heater resistors (heater resistor and power traces may be disposed in the surface above the ink feed channel).

A cross-section of a conventional printhead is shown in FIG. 1A. The conventional printhead is comprised of several individual layers of material constructed and assembled to perform its function. An orifice plate 100 forms the outermost layer of the printhead and is in close proximity of a printing medium. A plurality of heater resistors 102, more generally referred to as ink ejectors, is created by disposing resistive and conductive materials on the surface of a silicon wafer 104. An ink barrier layer 105 is selectively deposited on top of the silicon wafer 104 surface so that the inner walls 106, 108 form a firing chamber 110. In the conventional printhead, the ink barrier material is distinguished from the orifice plate material 100. Additionally, as shown in FIG. 1B, ink can only flow 112 into the firing chamber 110 from the perimeter of the heater resistor. This differs substantially from one embodiment of the present invention wherein ink may enter the firing chamber from the perimeter of the heater resistor and from beneath the heater resistor (ink feed channel is located directly beneath the heater resistor) as well. Once the conventional printhead has been fabricated, it is attached to an inkjet cartridge 200 at location 202 as shown in FIG. 2. The inkjet cartridge 200 is a fractionally hollow plastic housing comprising one or more ink containment components.

In accordance with a preferred embodiment of the current invention, ink feed channels 300 (as shown in FIG. 3a) are precisely manufactured in a substrate utilizing a two etch step micromachining technique. These ink feed channels serve as "ink inlets" for the printhead. FIG. 3B illustrates a variation of the printhead shown in FIG. 3A wherein the first etch of the aforementioned two etch step process removes a portion of the substrate where wall 312 remains. The second etch step removes a remaining portion (second portion) of the substrate, where wall 310 remains. Furthermore, the silicon ledge 316 created by the second etch process step provides structural support for a thinfilm material 314 that is formed on top of the substrate. The thinfilm material 314 contains an opening 318 that allows ink to flow from a reservoir to a heater resistor 302 as shown in FIG. 3C which is a top view of FIG. 3B. A detailed description of preferred embodiments and method of manufacture of the present invention is forthcoming:

FIG. 4A shows a silicon substrate 400 consisting of a first surface 402 and a second surface 404. The crystallographic orientation of the silicon wafer is <100> although <110> may be used. A multilayer insulating film (or dielectric film) 406 comprised of tetra ethyl ortho silicate TEOS, silicon nitride, and silicon carbide with an intervening dual layer conductor consisting of tantalum-aluminum and aluminum is formed on the first surface 402. The intervening conductive layer forms the heater resistor 302 (through the selective removal of one film) and the electrical lines 410 through which power is supplied to adjacent heater resistors (the heater resistor and electrical lines are shown pictorially). A

portion of a multilayer insulator hereinafter referred to as a thinfilm or thinfilm stack, is impervious to ink which may be corrosive. In this regard, the thinfilm protects the enclosed conductive layer 410, which is susceptible to ink corrosion.

A masking material (hard mask) which protects the second surface 404 of the substrate 400 from being undesirably etched, is formed on the second surface 404. This film may be formed of gate oxide, nitride, carbide, a polymer, a metal, or a combination thereof. Next, as shown in FIG. 4C the thinfilm 406 is patterned forming an opening 318 through which ink flows thereby reaching the heater resistor 302. This opening 318 determines the final dimensions of the ink feed channel.

FIG. 4D shows a polymer 416 formed on top of the thinfilm 406. The polymer forms a chamber 418 around the heater resistor (a "firing chamber") and defines an orifice 420 through which ink is ejected onto a printing medium. Additionally, the polymer provides structural support for the thinfilm. Next, the hard mask 403 formed on the second surface 404 is patterned and etched, thereby defining the location of the ink feed channel 500 as shown in FIG. 5A. The first portion of the etch is conducted using a conventional wet etch chemistry consisting of a diluted mixture of potassium hydroxide (KOH) or TMAH. In an embodiment of the current invention, the hard mask is formed before the polymer is formed.

The first portion of the wet etch anisotropically removes a predetermined amount 502 shown in the dashed area of FIG. 5A of the silicon substrate 400, thus, leaving the ink feed channel partially etched thereby forming syncline sidewalls 501 consistent with the crystallographic orientation of the substrate. The partially etched ink feed channel is covered with photoresist 504 as shown in FIG. 5C. The photoresist is applied to the ink feed channel using a conformal coating technique, which may include extrusion coating, spray coating or dipping. The photoresist 504 is then exposed in those areas 600 where the second portion of the ink feed channel etch will be performed (FIG. 6A). The second (and final) portion of the ink feed channel etch commences from the conclusion of the first etch. The second etch is preferably an anisotropic fluorine based plasma etch (dry etch). The fluorine-based plasma selectively etches a predetermined amount 602, shown in a dashed area of FIG. 6A, from the silicon substrate. Vertical sidewalls 601 are formed while leaving the thinfilm 406 unscathed as shown in FIG. 6B. FIG. 6C illustrates an embodiment of the present invention where the photoresist 504 has been removed.

Many embodiments of the current invention may be fabricated utilizing the aforementioned process including, but not limited to: (a) a printhead wherein ink may be filtered before reaching the heater resistor, (b) a printhead wherein heater resistors are disposed in the thinfilm directly above the ink feed channel, (c) a printhead wherein the first portion of the ink feed channel is sufficiently narrow thus causing the crystallographic planes to merge at a predetermined distance, (d) a printhead wherein the first portion of the ink feed channel etch is isotropic, (e) a printhead wherein a dopant or epitaxial layer is disposed between the first and second silicon surfaces forming an etch stop, and (f) a printhead wherein a commercially available silicon on oxide (SOI) substrate is utilized. A description of the aforementioned printheads embodying the current invention is described below:

(a) FIG. 7A shows an embodiment of the present invention wherein a grid 700 is created in the thinfilm 406 which serves to filter the ink (an ink filter) as it passes through the

ink feed channel in route to the heater resistor 302. If ink, being supplied to the ink filter, contains a particle of significant magnitude the particle may be trapped in the filter such that a portion of the ink feed channel remains open.

5 Additionally, the grid provides support for the thinfilm. This support is of great benefit for those configurations (as described below) where the heater resistor 302 resides above the ink feed channel. FIG. 7B shows an embodiment of the current invention wherein the second portion of the ink feed 10 channel has a segmented portion 704 forming sub-channels. This configuration increases the structural support of the printhead. Additionally, a plurality of heater resistors 302 may be disposed in the thinfilm 406 on either side of the segmented portion of the ink feed channel.

15 (b) FIG. 8A shows an embodiment of the current invention wherein the heater resistor is disposed in the thinfilm directly above the ink feed channel. In this configuration, ink may reach the heater resistor from both sides 800, 802 of the ink feed channel. This configuration also provides a means 20 for filtering the ink. For example, if opening 800 is clogged, ink may reach the heater resistor from opening 802. A multiplicity of heater resistors and accompanying nozzles (or orifices 420) may be disposed in a printhead employing this configuration, as shown in FIG. 8B. An embodiment as 25 such allows for high resolution printing (high DPI printing).

(c) FIG. 9A shows a printhead wherein the hard mask opening 500 is substantially narrowed. The final width chosen for the opening 500 allows the crystallographic planes to converge at point 902 at a predetermined distance 30 between the first surface 402 and the second surface 404 (FIG. 9A). An advantage of this technique is better control of the wet etched ink feed channel dimension. Since the planes inherently converge at 54.7 degrees, the dry etch will 35 repeatedly begin at the same depth, d, 904 into the substrate as shown in FIG. 9B.

(d) FIG. 10 shows a printhead wherein the first portion 40 of the ink feed channel etch is conducted using an isotropic chemical etch thereby forming an arch 1002 with concave walls. The isotropic characteristics of the etch stems 45 from the rate at which the substrate etches which is far greater than the anisotropic wet etch previously described. An advantage of the isotropic wet etching technique is a reduction in processing time. The previously described anisotropy wet etch process may take in excess of 15 hours to achieve whereas the isotropic etch may be achieved in less than five hours.

(e) FIG. 11A shows a printhead wherein the first surface 50 of the silicon substrate is doped to form a doped layer 1100 using a boron source in those regions where the ink feed channel is defined. The dopants are diffused into the substrate at a predetermined depth that creates an interface 1102 between the first surface 402 and the second surface 404. The aforementioned interface serves as an etch stop (the wet etch will not penetrate the doped surface interface) distinguishing the first etch (FIG. 11A) from the second etch (FIG. 11B). This technique lessens the need to time the etch, thus creating a more robust process. Additionally, it is possible to create a similar etch stop by growing a boron doped epitaxial layer on the first surface. The boron doped epitaxial layer will impede the wet chemical etch in a manner similar to the boron doped surface.

(f) FIG. 12A shows the printhead fabricated on a commercially available silicon on insulator substrate 1201 (commonly referred to as an SOI wafer). The intervening oxide layer 1200 between the first surface 402 and the second surface 404 (as shown in FIG. 12A) serves as an etch

stop. This etch stop is similar to that described previously, however, a silicon layer **1202** resides above the oxide layer **1200**. The ink feed channel is formed as described previously wherein the wet etch process is distinguished from the dry etch process by the intervening oxide layer **1200**. However, the dry etch process commences from the oxide interface **1203** (that is made visible following the wet etch process) and etches the silicon layer **1202** on top of the intervening oxide **1200** layer. The resulting embodiment is shown in FIG. 12B. Alternatively, the silicon layer **1202** on top of the intervening oxide layer **1200** may be etched subsequent to the time when the opening **318** in the thinfilm layer is etched. The advantage of this technique is the ability to utilize the inherent etch stop (oxide layer) of the wafer (starting material) to reduce processing time.

Many of the aforementioned challenges associated with the fabrication of ink feed channels have been remedied through an embodiments of the current invention including: (1) precise control of ink feed channel dimensions, (2) a decreased distance through which ink flows before reaching the heater resistor, (3) the manufacturing time of the printhead is reduced (as compared to a conventional printhead) and (4) greater packing density of the heater resistors disposed in the printhead thereby leading to greater print resolution. Various changes and modifications of an obvious nature may be made to an embodiment of the current invention without departing from the spirit of the invention and all such changes and modifications are considered to fall within the scope of the invention defined by the depending claims.

We claim:

1. A method of fabricating an ink feed channel for a thermal inkjet printhead comprising:

providing a substrate having at least one crystallographic orientation and at least two opposed planar surfaces with a first opposed planar surface and a second opposed planar surface;

etching a first portion of an ink feed channel commencing from said first opposed substrate surface and concluding between said at least two planar surfaces; and

etching a second portion of said ink feed channel commencing from the conclusion of said first etch to form a channel completely through said substrate and terminating at said second opposed planar surface, wherein etching said second portion of said ink feed channel includes using an anisotropic plasma dry etch.

2. The method of claim 1 wherein etching said first portion of said inkfeed channel includes using a wet anisotropic chemical etch.

3. The method of claim 1 further comprising disposing photoresist in partially completed inkfeed channel following said first etch.

4. The method according to claim 1 further comprising exposing said photoresist to form a pattern of said second portion of said ink feed channel.

5. The method of claim 1 further comprising:

disposing a dielectric film on the first opposed substrate surface; and

forming a pattern in said dielectric film disposed on said first opposed planar surface whereby an ink feed channel may be formed.

6. The method of claim 5 further comprising selecting said dielectric to be impervious to chemicals used to etch said substrate.

7. The method of claim 5 further comprising:

disposing a dielectric film on the second opposed substrate surface; and

terminating etching the second portion of said ink feed channel at said disposed dielectric film on the second opposed substrate surface.

5 8. The method of claim 7, further comprising forming an opening in said dielectric disposed on said second opposed substrate surface using a plasma dry etch, said opening being positioned above said inkfeed channel.

10 9. The method of claim 7, further comprising forming an opening in said dielectric disposed on said second opposed substrate surface using a wet chemical etch, said opening being positioned above said inkfeed channel.

15 10. The method of claim 1 further wherein said second portion of said inkfeed channel is narrower than said first portion.

15 11. The method of claim 1 wherein the first portion of the ink feed channel forms syncline sidewalls consistent with the crystallographic orientation of the substrate, wherein the crystallographic orientation is <100>.

20 12. A method of fabricating an ink feed channel for a thermal inkjet printhead comprising:

providing a substrate having at least one crystallographic orientation and at least two opposed planar surfaces with a first opposed planar surface and a second opposed planar surface;

etching a first portion of an ink feed channel commencing from said first opposed substrate surface and concluding between said at least two planar surfaces wherein the first portion of the ink feed channel forms sidewalls is consistent with the crystallographic orientation of the substrate, and wherein the crystallographic orientation is <110>; and

etching a second portion of said ink feed channel commencing from the conclusion of said first etch to form a channel completely through said substrate and terminating at said second opposed planar surface.

13. A method of fabricating an ink feed channel for a thermal inkjet printhead comprising:

providing a substrate having at least one crystallographic orientation and at least two opposed planar surfaces with a first opposed planar surface and a second opposed planar surface;

etching a first portion of an ink feed channel commencing from said first opposed substrate surface and concluding between said at least two planar surfaces wherein the first portion of the ink feed channel is etched through the substrate to an etch stop, wherein the etch stop is positioned in the substrate between the first and second opposed surfaces; and

etching a second portion of said ink feed channel commencing from the conclusion of said first etch to form a channel completely through said substrate and terminating at said second opposed planar surface.

14. A method of fabricating an ink feed channel for a thermal inkjet printhead comprising:

providing a substrate having at least one crystallographic orientation and at least two opposed planar surfaces with a first opposed planar surface and a second opposed planar surface;

forming an ink filter adjacent the second opposed planar surface;

etching a first portion of an ink feed channel, wherein the first portion is from said first opposed substrate surface to a location between said at least two planar surfaces; and

**9**

etching a second portion of said ink feed channel, wherein the second portion of the channel is from the location between said at least two planar surfaces to said second opposed substrate surface.

**15.** The method of claim **14** wherein the ink is filtered before it reaches a heater resistor formed directly above the ink feed channel.

**16.** The method of claim **14** further comprising a dielectric layer deposited over the substrate, wherein the dielectric layer has a plurality of holes over the ink feed channel thereby forming the ink filter.

**17.** The method of claim **14** further comprising etching the second portion of the ink feed channel into segments thereby forming subchannels, wherein the subchannels are the ink filter.

**18.** A method of fabricating an ink feed channel for a thermal inkjet printhead comprising:

**10**

providing a substrate having at least one crystallographic orientation and at least two opposed planar surfaces with a first opposed planar surface and a second opposed planar surface;

etching a first portion of an ink feed channel commencing from said first opposed substrate surface and concluding between said at least two planar surfaces, wherein the first portion is formed as an arch; and

etching a second portion of said ink feed channel commencing from the conclusion of said first etch to form a channel completely through said substrate and terminating at said second opposed planar surface.

**19.** The method of claim **18** further comprising forming the arch using an isotropic chemical etch.

\* \* \* \* \*